# EUROPEAN PATENT SPECIFICATION

(11) **EP 3 666 919 B1**
(45) Date of publication and mention of the grant of the patent: **08.11.2023**
(21) Application number: 18845253.6
(22) Date of filing: 03.08.2018
(51) Int. Cl.: C22C 38/14, C22C 38/04, C22C 38/06, C22C 38/02, C21D 8/02, C21D 9/46, C23C 2/06, C23C 2/02, C23C 30/00

(54) **PLATED STEEL SHEET HAVING EXCELLENT SURFACE QUALITY, STRENGTH AND DUCTILITY**
PLATTIERTES STAHLBLECH MIT HERVORRAGENDER OBERFLÄCHENQUALITÄT, FESTIGKEIT UND DUKTILITÄT
TÔLE D'ACIER PLAQUÉE AYANT UNE EXCELLENTE QUALITÉ DE SURFACE, UNE EXCELLENTE RÉSISTANCE ET UNE EXCELLENTE DUCTILITÉ

(30) Priority: 09.08.2017 KR 20170101268
(43) Date of publication of application: 17.06.2020
(73) Proprietor: POSCO Co., Ltd, Pohang-si, Gyeongsangbuk-do 37859 (KR)
(72) Inventor: KIM, Yong-Woo, Pohang-si Gyeongsangbuk-do 37877 (KR)
(74) Representative: Meissner Bolte Partnerschaft mbB
(86) International application number: PCT/KR2018/008848
(87) International publication number: WO 2019/031773

(56) References cited:
- JP-A- 2010 144 242
- JP-A- 2014 095 146
- JP-A- 2014 095 146
- KR-A- 20140 138 854
- KR-A- 20150 029 742
- KR-B1- 101 033 752
- US-A1- 2008 202 639
- US-A1- 2013 319 582
- US-A1- 2015 284 819

## Description

### [Technical Field]

The present invention relates to a plated steel sheet having excellent surface quality, strength, and ductility, and more particularly, to a plated steel sheet having excellent surface quality, strength, and ductility, which may be preferably used as a pre-engineered building (PEB) structure.

### [Background Art]

The PEB method may be a method that minimizes the use of materials through optimal design, considering the supporting load, and may be a construction method capable of reducing construction costs and shortening a construction period. The PEB structure used in the PEB method may be required to have excellent strength in order to prevent buckling by load, and the like. Therefore, a steel sheet conventionally used as the PEB structure may be generally manufactured by adding C, Si, Mn, Ti, Nb, Mo, V, and the like to a high purity steel having minimized impurities therein.

Typically, a method of utilizing precipitation strengthening of the following elements by adding Ti, Nb, V, Mo, and the like (Patent Document 1, Patent Document 2), a method of securing strength by adding a relatively large amount of Cr, Mn, or the like (Patent Document 3, Patent document 4), and a method of increasing impact strength and tensile characteristics by temper annealing Mn and Cr-added steel (patent document 5), and the like have been known. US2013 03 19582 A1 describes a bainite-containing-type hot-rolled steel sheet.

In addition, the construction industry in recent years has sought to process a thin material to a shape more due to the change of the design of the structure for reducing costs. Therefore, in order to cope with such a market situation, steel sheets having excellent ductility as well as strength are required. However, the conventional techniques presented above focus only on an increase in strength through solid solution strengthening by alloy components such as C, Si, Mn, Cr, Mo, W, and the like, and precipitation strengthening by alloy components such as Ti, Nb, Mo, and the like. Therefore, there is a limit to ductility improvement.

Meanwhile, since the PEB structure is required to have excellent corrosion resistance, a plating film may be generally formed on the surface of the steel sheet used as the PEB structure. Therefore, in the case of the steel sheet used as the PEB structure, the surface quality of the hot-rolled steel sheet before performing a plating process becomes a very important factor. In the case of the conventional techniques presented above, the alloy material may be relatively excessive, and the hot-rolling resistance may be relatively high. Therefore, in producing thin sheets having less than 2.0t thickness, there may be a problem that the plating quality is deteriorated due to occurrence of sand-type scales by a hot-rolling process.

### [Related Prior Arts]

### (Patent Documents)

(Patent Document 1) Japanese Patent Publication No. 2011-102434
(Patent Document 2) Japanese Patent Publication No. 2004-359974
(Patent Document 3) European Patent Publication No. 1375694
(Patent Document 4) Korean Patent Publication No. 1997-7002384
(Patent Document 5) International Patent Publication No. 2011-154831
(Patent Document 6) US 2013 0319582 A1

### [Disclosure]

### [Technical Problem]

The present invention provides a plated steel sheet having excellent surface quality, strength, and ductility, and a method of manufacturing the same.

### [Technical Solution]

Solution to the technical problem above is provide in the claims.

### [Advantageous Effects]

As one of several effects of the present invention, the plated steel sheet according to the present invention may have the advantages not only of excellent surface quality, such as no surface defects, but also excellent balance of yield strength and elongation.

Various and advantageous advantages and effects of the present invention are not limited to the above description, it will be more readily understood in the course of describing specific embodiments of the present invention.

### [Description of Drawings]

The above and other aspects, features, and advantages of the present invention will be more clearly understood from the following detailed description, taken in conjunction with the accompanying drawings, in which:
(a) of FIG. 1 is a photograph of a surface of a plated steel sheet of Comparative Example 2, and (b) of FIG. 1 is a photograph of a surface of a plated steel sheet of Inventive Example 1.
FIG. 2 is a graph illustrating elongation to yield strength of the Inventive and Comparative Examples.

### [Best Mode for Invention]

Hereinafter, a plated steel sheet having excellent surface quality, strength, and ductility as an aspect of the present invention will be described in detail.

A plated steel sheet having excellent surface quality, strength, and ductility, which is one aspect of the present invention, includes a hot-rolled steel sheet, and a plating film formed on a surface of the hot-rolled steel sheet. The plating film includes, but is not necessarily limited to, Mg: 10% or less, Al: 5% or less, a balance of Zn, and inevitable impurities.

Hereinafter, alloying element and preferred content ranges of the hot-rolled steel sheet will be described in detail. It is to be noted that the content of each element described below may be based on weight unless otherwise specified.

### Carbon (C) : 0.15 - 0.25%

C may be the most economical and effective element for securing strength. When the C content is too low, it may be difficult to secure the target strength. Therefore, the C content is 0.15% or more, and it is preferable that the C content is 0.16% or more. When the content is overly excessive, ductility may be deteriorated due to an excessive increase in strength. Therefore, the C content is 0.25% or less, and preferably 0.22% or less.

### Silicon (Si): 0.5% or less

Si may contribute to an increase in strength due to solid solution strengthening and deoxidation of molten steel, but may be not intentionally added in the present invention. Even when Si is not added, there may be no major problem in terms of securing physical properties. When the content is overly excessive, red scale due to Si may be formed on the surface of the hot-rolled steel sheet. Therefore, surface quality and plating quality may be deteriorated. In some cases, the Si content may exclude 0%.

### Manganese (Mn) : 0.5 - 2.0%

Mn may be an effective element for solute strengthening of steel, and needs to be 0.5% or more, preferably 0.6% or more to secure appropriate strength. When the content is excessively large, there may be a risk that a central segregation portion occurs in the continuous casting process. Therefore, the Mn content is 2.0% or less, and it is preferable that the Mn content is 1.8% or less.

### Phosphor (P): 0.03% or less

P may be an inevitable impurity contained in steel, and it is preferable to control its content as low as possible. In particular, when the content is excessive, the risk of weldability deterioration and brittleness of the steel may increase. Therefore, in the present invention, the P content is managed to be 0.03% or less. In some cases, the P content may exclude 0%.

### Sulfur (S): 0.015% or less

S may be an impurity that may be inevitably included in steel, and it is preferable to control its content as low as possible. In particular, when the content is excessive, it may be combined with Mn to form a non-metallic inclusion, and the risk of brittleness of the steel may increase. Therefore, in the present invention, the content is managed to be 0.015% or less. In some cases, the S content may exclude 0%.

### Aluminum (Al): 0.05% or less

Al may contribute to deoxidation of molten steel, but may be not intentionally added in the present invention. Even when Al is not added, there may be no major problem in terms of securing physical properties. When the content is excessive, nozzle clogging, and the like may occur in the continuous casting process. In the present invention, the content is managed to be 0.05% or less. In some cases, the Al content may exclude 0%.

### Nitrogen (N) : 0.01% or less

N may contribute to improvements in strength of steel, but in the present invention may be not added intentionally. Even when N is not added, there may be no major problem in terms of securing physical properties. When the content is excessive, the risk of brittleness of the steel may increase. Therefore, in the present invention, the content is managed to be 0.01% or less. In some cases, the N content may exclude 0%.

### Titanium (Ti): 0.01 to 0.05%

Ti may be present in steel as TiN, to suppress growth of crystal grains during a heating operation for hot-rolling. In addition, it may serve to remove N, such that B does not react with N. When the content is excessive, there may be a risk of clogging the nozzle during the continuous casting process due to excessive TiN precipitation. Therefore, the Ti content is 0.05% or less, preferably 0.04% or less, and more preferably 0.03% or less. Further, since Ti needs to be added to steel to obtain the above-mentioned effect, the lower limit of the Ti content is limited to 0.01% in terms of securing a sufficient crystal grain growth inhibiting effect.

### Boron (B): 0.0005 to 0.01%

B may be contained as an alternative element of Si, improve quenchability in very small amounts, and strengthen grain boundaries to improve strength. When the content is excessive, there may be a risk of surface quality deterioration due to excessive BN precipitation. Therefore, the B content is 0.01% or less, preferably 0.008% or less, and more preferably 0.005% or less. Further, since B needs to be added to steel to obtain the above-mentioned effect, the lower limit of the B content is limited to 0.0005%, preferably 0.001% in terms of securing sufficient quenchability.

In addition to the above composition, the rest is Fe. In the usual manufacturing process, since inevitable impurities that may be not intended from the raw materials or the surrounding environment may be inevitably mixed, these cannot be excluded. Since these impurities are known to those skilled in the art, not all of them may be specifically mentioned in the present specification.

When designing alloy of steel having component ranges as described above, it is preferable to control to satisfy the following relationship 1. The relationship 1 below may be a factor of surface quality of the steel sheet. When the relationship 1 is satisfied, the finish temperature of hot-rolling may be secured to less than 900°C thanks to the reduction of the hot-rolling resistance. Therefore, since sand-type scale, which is generated by a high temperature during hot-rolling, is not generated, it is possible to secure a plated steel sheet having excellent surface quality after a final plating operation. When the relationship 1 is not satisfied, sand-type scale may be generated due to the high temperature during the hot-rolling operation, and plating quality may be degraded. $\begin{matrix}0.235 \left[C\right] + 0.0158 \left[Mn\right] + 0.0625 \left[Si\right] + 0.0423 \left[Mo\right] + 0.317 \left[Ti\right] \\ + 1.36 \left[Nb\right] \leq 0.075\end{matrix}$

Where [C], [Mn], [Si], [Mo], [Ti], and [Nb] represent the content (by wt%) of the corresponding elements contained in the steel sheet, respectively.

Hereinafter, a microstructure of the steel sheet will be described in detail.

The hot-rolled steel sheet, which is the base of the plated steel sheet of the present invention, comprises, by area, 10 to 30% of ferrite, 20 to 40% of pearlite, and 35 to 55% of bainite, and more preferably 15 to 25% of ferrite, 25 to 35% of pearlite, and 40 to 50% of bainite, as a microstructure. When phase fractions as described above are not secured, it may be difficult to secure a balance of target strength and ductility due to a decrease in strength or ductility. According to an embodiment of the present invention, the sum of the fractions of ferrite, pearlite, and bainite may be 90 area% or more.

According to an example, an average grain size of the ferrite may be 20 um or less (excluding 0 µm), and more preferably 15 um or less (excluding 0 um) . When the average grain size of the ferrite exceeds 20um, it may be difficult to secure the desired strength. The smaller the average grain size of the ferrite, the more advantageous for securing strength. Therefore, the lower limit thereof is not particularly limited in the present invention. In this case, the grain size refers to an equivalent circular diameter of particles detected by observing one cross section of the steel.

According to an example, an average colony size of pearlite may be 30 um or less (excluding 0 µm), and more preferably 20 um or less (excluding 0 um) . When the colony size of pearlite exceeds 30um, it may be difficult to secure a desired combination of strength x ductility due to inferior ductility, and in particular, cracking may occur due to deterioration of bendability during the manufacture of final product. The smaller the average colony size of pearlite, the more advantageous for securing strength. Therefore, the lower limit thereof is not particularly limited in the present invention. In this case, the colony size refers to an equivalent circular diameter of particles, divided by tilt boundaries having misorientation angle of 15 degrees or more detected by observing the inside of pearlite.

In the present invention, residual structure, other than the ferrite, pearlite, and bainite, is not particularly limited, and in some cases, may be further include at least one second phase of martensite, cementite, and residual austenite. All of these second phases may be hard phases. When the area ratio of these second phases is too high, the combination of strength x ductility may be deteriorated, because the strength is relatively high and the ductility is relatively low. The sum of these area ratios may be controlled to be preferably 10% or less, more preferably 5% or less.

Plated steel sheet of the present invention may have a relatively high yield strength, and, according to an example, may have a yield strength of 450 - 600MPa.

In addition, the plated steel sheet of the present invention may have the advantage of excellent balance of strength and ductility, and, according to an example, the product of yield strength and elongation may be 8,500MPa·% or more.

Hereinafter, a method of manufacturing a plated steel sheet having excellent strength and ductility of the present invention will be described in detail.

First, a slab having the above-described composition system is reheated at 1100 to 1300°C. When the reheating temperature is less than 1100°C, the rolling load may be too large in a subsequent hot-rolling process. When the reheating temperature is higher than 1300°C, austenite grains may be partially coarsened due to abnormal growth of some austenite grains, such that the grain size of the final microstructure may be not homogeneous. In addition, in the present invention, slab reheating time is not specifically limited, and is acceptable under normal conditions. In a non-limiting example, the slab reheating time may be 100 to 400 minutes.

Next, after rough-rolling the reheated slab, the rough-rolled slab is finish-rolled at the austenite single phase temperature (temperature of Ar3°C or higher), to obtain a hot-rolled steel steel. In this case, rough-rolling refers to a series of intermediate rolling processes performed before finish-rolling. In addition, in the present invention, the rough-rolling is not specifically limited, and is acceptable under normal conditions. In a non-limiting example, a thickness of the rough-rolled slab relative to a thickness of the reheated slab may be 10 to 25%, and the rough-rolling temperature may be set to a sufficiently high temperature at which the finish-rolling temperature is ensured.

According to the present invention, the finish-rolling is carried out in the range of (FDT-20) °C to (FDT+20) °C defined by the following equation 2. When the finish rolling temperature exceeds FDT+20°C, austenitic grains of the slab may be coarsened such that sizes of the final ferrite grains and pearlite colonies may be coarse, leading to a decrease in strength. Therefore, it may be difficult to secure desired excellent strength x ductility. When the finish-rolling temperature is less than FDT-20°C, mixed-grain structure may be generated due to two phase temperature rolling, to reduce the ductility, and rolling load may greatly increase during hot-rolling, to decrease productivity. In addition, the mixed-grain structure refers that crystal grains having different particle sizes are mixed. When finish-rolling in the above temperature range, the austenitic structure of the hot finish-rolled steel sheet has an average grain size of 10 - 40um. $\begin{matrix}FDT \left(°C\right) = 1002.1 - 353 \left[C\right] + 43.9 \left[Si\right] - 74.1 \left[Mn\right] - 20.4 \left[Cu\right] - 19 \\ .9 \left[Cr\right] - 45.6 \left[Ni\right] - 80 \left[Mo\right]\end{matrix}$

Where [C], [Si], [Mn], [Cu], [Cr], [Ni], and [Mo] represent the content (by wt%) of the corresponding elements contained in the steel sheet, respectively.

Next, the hot-rolled steel sheet is cooled at a cooling rate of Vc°C/s or more and (Vc+30) °C/s or less, defined by the following equation 1, and is then coiled. When the cooling rate is less than Vc°C/s, it may be difficult to secure the desired strength, because the fraction of ferrite and pearlite exceeds the range limited by the present invention. When the cooling rate exceeds (Vc+30) °C/s, the fraction of bainite or second phase may exceed the limit of the present invention, to deteriorate the ductility. Therefore, a combination of excellent (yield strength x ductility) may be not be obtained. $\begin{matrix}Vc = 158.0 - 156.6 \left[C\right] + 246.6 \left[Si\right] - 40.32 \left[Mn\right] - 25.74 \left[Cr\right] - 73 . \\ 26 \left[Ni\right] - 8820 \left[B\right] - 1483.2 \left[Ti\right] + 1108.8 \left[Nb\right] - 291.6 \left[Mo\right] - 1092.6 \left[V\right]\end{matrix}$

Where [C], [Si], [Mn], [Cr], [Ni], [B], [Ti], [Nb], [Mo], and [V] represent the content (by wt%) of the corresponding elements contained in the steel sheet, respectively.

According to the present invention, the coiling is carried out in a range of (CT-20) °C to (CT+20) °C defined by the following equation 3. When the coiling temperature exceeds (CT+20)°C, coarse ferrite and pearlite may be formed to lower yield strength. Therefore, the desired (yield strength x elongation) value may be not be obtained. When the coiling temperature is less than CT-20°C, ductility may be deteriorated. More specifically, when the coiling temperature is less than CT-20°C, bainite may be excessively formed beyond the fraction of the present invention to cause the ductility deteriorated while making the yield strength increase. Therefore, the desired (yield strength x elongation) value may be not be obtained. Therefore, when controlling and cooling the coiling temperature in the above temperature range, it is possible to obtain a hot-rolled steel sheet having a preferred microstructure, proposed by the present invention. $\begin{matrix}CT = 751.7 - 357.3 \left[C\right] - 85.3 \left[Mn\right] - 35 \left[Si\right] - 73 \left[Cr\right] - 36 \left[Ni\right] - 84 . \\ 4 \left[Mo\right]\end{matrix}$

Where [C], [Mn], [Si], [Cr], [Ni], and [Mo] represent the content (by wt%) of the corresponding elements contained in the steel sheet, respectively.

Next, hot-dip plating process of the coiled hot-rolled steel sheet is followed. The hot-dip plating process according to an embodiment of the present invention may be carried out by hot-dip plating a solution comprising, by weight, Mg: 10% or less, Al: 5% or less, a balance of Zn, and inevitable impurities.

### [Mode for Invention]

Hereinafter, the present disclosure will be described in more detail with reference to examples. However, the description of these examples may be only for illustrating the practice of the present invention, and the present invention is not limited by the description of these examples. This may be because the scope of the present invention may be determined by the matters described in the claims and the matters reasonably inferred therefrom.

### (Example)

A steel slab having a component system described in the following Table 1 (the contents of P and S as impurities in each steel were controlled at 0.03% by weight or less and 0.015% by weight or less, respectively, the Cu content was 0% by weight, and the N content was 0.005% by weight) was heated to 1200°C, and finish-rolling was performed at the hot finish-rolling temperature shown in the following Table 2, to obtain a hot-rolled steel sheet. Thereafter, the hot-rolled steel sheet was cooled to the coiling temperature described in the following Table 2 at a cooling rate (CR, °C/s), and then coiled up. Thereafter, the coiled hot-rolled steel sheet was subjected to hot-dip plating.

Then, a microstructure of the plated steel sheet thus-prepared was analyzed, mechanical properties were evaluated, and results therefrom were shown in the following Table 3. In the microstructure of the following Table 3, F refers to ferrite, P refers to pearlite, B refers to bainite, and among grain size, F refers to an average grain size of ferrite, P refers to an average colony size of pearlite, and among mechanical properties, YP refers to yield strength, TS refers to tensile strength, and El refers to elongation.

In addition, surface quality after plating was visually measured, and results therefrom were shown in the following Table 3. A case in which surface defects such as scales or tear marks were detected is evaluated to be "X", and a case in which surface defects were not detected is evaluated to be "O".

**[Table 1]**

| Type of Steel | Alloy Composition (wt%) | | | | | | | | | | | R1*** |
|---|---|---|---|---|---|---|---|---|---|---|---|---|
| | C | Si | Mn | s.Al | Cr | Ni | B | Ti | Nb | Mo | V | |
| IS1* | 0.18 | 0.06 | 1.1 | 0.035 | 0 | 0 | 0.0015 | 0.025 | 0 | 0 | 0 | 0.071 |
| IS2 | 0.17 | 0.06 | 1.1 | 0.035 | 0 | 0 | 0.0015 | 0.025 | 0 | 0 | 0 | 0.069 |
| IS3 | 0.19 | 0.06 | 1.1 | 0.035 | 0 | 0 | 0.0015 | 0.025 | 0 | 0 | 0 | 0.074 |
| IS4 | 0.18 | 0.06 | 1.05 | 0.035 | 0 | 0 | 0.0015 | 0.025 | 0 | 0 | 0 | 0.071 |
| IS5 | 0.18 | 0.06 | 1.15 | 0.035 | 0 | 0 | 0.0015 | 0.025 | 0 | 0 | 0 | 0.072 |
| IS6 | 0.18 | 0.06 | 1.1 | 0.035 | 0 | 0 | 0.001 | 0.025 | 0 | 0 | 0 | 0.071 |
| IS7 | 0.18 | 0.06 | 1.1 | 0.035 | 0 | 0 | 0.0018 | 0.025 | 0 | 0 | 0 | 0.071 |
| IS8 | 0.18 | 0.06 | 1.1 | 0.035 | 0 | 0 | 0.0015 | 0.022 | 0 | 0 | 0 | 0.070 |
| IS9 | 0.18 | 0.06 | 1.1 | 0.035 | 0 | 0 | 0.0015 | 0.028 | 0 | 0 | 0 | 0.072 |
| CS1** | 0.22 | 0 | 0.8 | 0.035 | 0 | 0 | 0.0015 | 0 | 0 | 0 | 0 | 0.064 |
| CS2 | 0.22 | 0.06 | 1 | 0.035 | 0 | 0 | 0.0015 | 0.025 | 0 | 0 | 0 | 0.079 |
| CS3 | 0.16 | 0.06 | 1.1 | 0.035 | 0 | 0 | 0.0015 | 0 | 0.02 | 0 | 0 | 0.086 |
| CS4 | 0.16 | 0.06 | 1.3 | 0.035 | 0 | 0 | 0 | 0 | 0 | 0 | 0 | 0.062 |
| CS5 | 0.18 | 0.06 | 1.1 | 0.035 | 0 | 0 | 0.0015 | 0.025 | 0 | 0 | 0 | 0.071 |

| | | | | | | | | | | | | |
|---|---|---|---|---|---|---|---|---|---|---|---|---|
| *IS: Inventive Steel, **CS: Comparative Steel, ***R: Relationship | | | | | | | | | | | | |

**[Table 2]**

| Type of Steel | Ar3 | FDT(°C) | Finish-Rolling Temp. (°C) | CT(°C) | Coiling Temp. (°C) | Vc (°C/sec) | CR (°C/sec) | Remark |
|---|---|---|---|---|---|---|---|---|
| IS1* | 772 | 860 | 870 | 591 | 580 | 50 | 55 | IE1*** |
| IS2 | 775 | 863 | 870 | 595 | 580 | 52 | 57 | IE2 |
| IS3 | 769 | 856 | 860 | 588 | 580 | 48 | 53 | IE3 |
| IS4 | 776 | 863 | 870 | 596 | 580 | 52 | 57 | IE4 |
| IS5 | 768 | 856 | 865 | 587 | 580 | 48 | 53 | IE5 |
| IS6 | 772 | 860 | 870 | 591 | 580 | 54 | 59 | IE6 |
| IS7 | 772 | 860 | 870 | 591 | 580 | 47 | 52 | IE7 |
| IS8 | 772 | 860 | 870 | 591 | 580 | 54 | 59 | IE8 |
| IS9 | 772 | 860 | 870 | 591 | 580 | 45 | 50 | IE9 |
| CS1** | 784 | 865 | 870 | 605 | 590 | 78 | 70 | CE1**** |
| CS2 | 768 | 853 | 900 | 586 | 580 | 48 | 53 | CE2 |
| CS3 | 778 | 867 | 900 | 599 | 580 | 112 | 70 | CE3 |
| CS4 | 762 | 852 | 860 | 582 | 580 | 95 | 70 | CE4 |
| CS5 | 772 | 860 | 870 | 591 | 520 | 50 | 55 | CE5 |
| IS1 | 772 | 860 | 750 | 591 | 580 | 50 | 55 | CE6 |
| IS1 | 772 | 860 | 870 | 591 | 580 | 50 | 30 | CE7 |
| IS2 | 775 | 860 | 875 | 595 | 580 | 48 | 40 | CE8 |

| | | | | | | | | |
|---|---|---|---|---|---|---|---|---|
| *IS: Inventive Steel, **CS: Comparative Steel, ***IE: Inventive Example, ****CE: Comparative Example | | | | | | | | |

**[Table 3]**

| Remark | Surface Quality | Microstructure (area%) | | | Grain Size (um) | | Mechanical Properties | | | |
|---|---|---|---|---|---|---|---|---|---|---|
| | | F | P | B | F | P | YP (MPa) | TS (MPa) | EL (%) | YP* EL |
| IE1* | ○ | 20 | 30 | 45 | 9 | 12 | 510 | 615 | 18.5 | 9440 |
| IE2 | ○ | 22 | 29 | 44 | 10 | 13 | 496 | 604 | 18.7 | 9281 |
| IE3 | ○ | 18 | 31 | 46 | 9 | 11 | 525 | 626 | 18.3 | 9594 |
| IE4 | ○ | 22 | 29 | 43 | 11 | 14 | 493 | 602 | 18.7 | 9216 |
| IE5 | ○ | 18 | 31 | 47 | 9 | 9 | 528 | 629 | 18.3 | 9657 |
| IE6 | ○ | 25 | 29 | 42 | 14 | 13 | 471 | 584 | 19.1 | 8982 |
| IE7 | ○ | 17 | 31 | 47 | 8 | 7 | 534 | 634 | 18.1 | 9693 |
| IE8 | ○ | 25 | 28 | 41 | 13 | 14 | 470 | 584 | 19.1 | 8977 |
| IE9 | ○ | 15 | 32 | 49 | 8 | 6 | 551 | 647 | 17.9 | 9855 |
| CE1** | ○ | 37 | 25 | 33 | 15 | 15 | 376 | 511 | 20.2 | 7602 |
| CE2 | X | 18 | 31 | 47 | 22 | 36 | 529 | 629 | 18.1 | 9592 |
| CE3 | X | 37 | 25 | 33 | 21 | 32 | 374 | 510 | 20.5 | 7676 |
| CE4 | ○ | 20 | 30 | 45 | 11 | 17 | 373 | 508 | 20.7 | 7730 |
| CE5 | ○ | 20 | 15 | 60 | 12 | 13 | 615 | 698 | 11.2 | 6888 |
| CE6 | ○ | 50 | 30 | 15 | 15 | 17 | 400 | 570 | 23.1 | 9240 |
| CE7 | ○ | 40 | 45 | 10 | 12 | 16 | 420 | 590 | 21.4 | 8988 |
| CE8 | ○ | 45 | 33 | 17 | 13 | 17 | 380 | 550 | 24.2 | 9196 |

| | | | | | | | | | | |
|---|---|---|---|---|---|---|---|---|---|---|
| *IE: Inventive Example, **CE: Comparative Example | | | | | | | | | | |

As may be seen from Table 3, Inventive Examples 1 to 9 satisfying all of the alloy composition and manufacturing conditions proposed by the present invention had excellent surface quality due to no surface defects. In addition, the product of yield strength and elongation was 8,500 MPa·% or more. Therefore, balance between strength and ductility was excellent.

On the other hand, in the case of Comparative Examples 1 and 4, the cooling rate CR was lower than the limit of the present invention and the ferrite fraction was high. Therefore, the yield strength was lowered, and the product of yield strength and elongation was deteriorated.

In the case of Comparative Example 2, the relationship 1 exceeded the defined ranges of the present invention and the hot finish-rolling temperature (FDT) exceeded the defined ranges of the present invention. Therefore, the plated surface was deteriorated by the occurrence of surface defects due to the scale.

In the case of Comparative Example 3, the relationship 1 and the cooling rate were both outside the defined ranges of the present invention. Therefore, the surface quality was also deteriorated, and the product of yield strength and elongation was also deteriorated.

In the case of Comparative Example 5, the coiling temperature was beyond the defined ranges of the present invention, the strength was excessively high. Therefore, the elongation was deteriorated, and as a result, the product of yield strength and elongation was deteriorated.

In the case of Comparative Example 6, the alloy composition satisfies the defined ranges of the present invention, but when the finish rolling temperature was lower than Ar3, the ferrite fraction was excessively produced during rolling. Therefore, sufficient yield strength could not be obtained.

Comparative Examples 7 and 8 may be cases in which the cooling rate did not satisfy the ranges defined by the present invention. As a result, the fractions of ferrite and pearlite were higher than the value to be controlled by the present invention, and the yield of bainite was low. Therefore, sufficient yield strength could not be obtained.

Portion (a) in FIG. 1 is a photograph of a surface of a plated steel sheet of Comparative Example 2, and portion (b) in FIG. 1 is a photograph of a surface of a plated steel sheet of Inventive Example 1. FIG. 2 is a graph illustrating elongation to yield strength of the Inventive and Comparative Examples.

## Claims

1. A plated steel sheet having a plating film on a surface of a hot-rolled steel sheet, wherein the hot-rolled steel sheet comprises, by weight, 0.15 to 0.25% of C, 0.5% or less of Si, 0.5 to 2.0% of Mn, 0.03% or less of P, 0.015% or less of S, 0.05% or less of Al, 0.01% or less of N, 0.01 to 0.05% of Ti, 0.0005 to 0.01% of B, a balance of Fe, and inevitable impurities,
wherein the elements satisfy the following relationship 1, and
wherein the hot-rolled steel sheet comprises, by area, 10 to 30% of ferrite, 20 to 40% of pearlite, and 35 to 55% of bainite, as a microstructure, $0.235 \left[C\right] + 0.0158 \left[Mn\right] + 0.0625 \left[Si\right] + 0.0423 \left[Mo\right] + 0.317 \left[Ti\right] + 1.36 \left[Nb\right] \leq 0.075 ,$
wherein [C], [Mn], [Si], [Mo], [Ti], and [Nb] represent the content of the corresponding elements contained in the steel sheet in wt%, respectively.

2. The plated steel sheet according to claim 1, wherein a sum of the fractions of the ferrite, pearlite, and bainite is 90 area% or more.

3. The plated steel sheet according to claim 1, wherein an average grain size of the ferrite is 20µm or less excluding 0µm.

4. The plated steel sheet according to claim 1, wherein an average colony size of the pearlite is 30µm or less excluding 0µm.

5. The plated steel sheet according to claim 1, wherein the plating film comprises, by weight, 10% or less of Mg, 5% or less of Al, a balance of Zn, and inevitable impurities.

6. The plated steel sheet according to claim 1, wherein the plated steel sheet has a yield strength of 450 to 600MPa.

7. The plated steel sheet according to claim 1, wherein a product of a yield strength and an elongation of the plated steel sheet is 8,500MPa·% or more.

8. The plated steel sheet according to claim 1, wherein the hot-rolled steel sheet is a thin material of less than 2.0mm sheet thickness.

9. A method for manufacturing a plated steel sheet, comprising:
reheating a slab comprising, by weight, 0.15 to 0.25% of C, 0.5% or less of Si, 0.5 to 2.0% of Mn, 0.03% or less of P, 0.015% or less of S, 0.05% or less of Al, 0.01% or less of N, 0.01 to 0.05% of Ti, 0.0005 to 0.01% of B, a balance of Fe, and inevitable impurities, to 1100 to 1300°C, wherein the elements satisfy the following relationship 1;
finish-rolling the reheated slab to a temperature of Ar3°C or higher to obtain a hot-rolled steel sheet;
cooling the hot-rolled steel sheet at a rate of Vc to (Vc+30)°C/s defined by the following equation 1, and coiling the cooled hot-rolled steel sheet; and
hot-dip plating by dipping the coiled hot-rolled steel sheet in a hot-dip bath,
wherein the finish-rolling is carried out in a range of (FDT-20)°C to (FDT+20)°C defined by the following equation (2), and
wherein the coiling is carried out in a range of (CT-20)°C to (CT+20)°C defined by the following equation 3, $0.235 \left[C\right] + 0.0158 \left[Mn\right] + 0.0625 \left[Si\right] + 0.0423 \left[Mo\right] + 0.317 \left[Ti\right] + 1.36 \left[Nb\right] \leq 0.075 ,$
wherein [C], [Mn], [Si], [Mo], [Ti], and [Nb] represent the content of the corresponding elements contained in the steel sheet in wt%, respectively, $\begin{matrix}Vc = 158.0 - 156.6 \left[C\right] + 246.6 \left[Si\right] - 40.32 \left[Mn\right] - 25.74 \left[Cr\right] - 73.26 \left[Ni\right] - 8820 \left[B\right] - \\ 1483.2 \left[Ti\right] + 1108.8 \left[Nb\right] - 291.6 \left[Mo\right] - 1092.6 \left[V\right] ,\end{matrix}$
wherein [C], [Si], [Mn], [Cr], [Ni], [B], [Ti], [Nb], [Mo], and [V] represent the content of the corresponding elements contained in the steel sheet in wt%, respectively, $FDT \left(°C\right) = 1002.1 - 353 \left[C\right] + 43.9 \left[Si\right] - 74.1 \left[Mn\right] - 20.4 \left[Cu\right] - 19.9 \left[Cr\right] - 45.6 \left[Ni\right] - 80 \left[Mo\right] ,$
wherein [C], [Si], [Mn], [Cu], [Cr], [Ni], and [Mo] represent the content of the corresponding elements contained in the steel sheet in wt%, respectively, $CT = 751.7 - 357.3 \left[C\right] - 85.3 \left[Mn\right] - 35 \left[Si\right] - 73 \left[Cr\right] - 36 \left[Ni\right] - 84.4 \left[Mo\right] ,$
wherein [C], [Mn], [Si], [Cr], [Ni], and [Mo] represent the content of the corresponding elements contained in the steel sheet in wt%, respectively.

10. The method according to claim 9, wherein the hot-dip bath comprises, by weight, 10% or less of Mg, 5% or less of Al, a balance of Zn, and inevitable impurities.

## Patentansprüche

1. Beschichtetes Stahlblech mit einer Plattierungsschicht auf einer Oberfläche eines warmgewalzten Stahlblechs, wobei das warmgewalzte Stahlblech in Gewicht 0,15 bis 0,25% an C, 0,5% oder weniger an Si, 0,5 bis 2,0 % an Mn, 0,03% oder weniger an P, 0,015% oder weniger an S, 0,05% oder weniger an AI, 0,01% oder weniger an N, 0,01 bis 0,05% an Ti, 0,0005 bis 0,01% an B, einen Rest an Eisen und unvermeidbare Verunreinigungen umfasst, wobei die Elemente das folgende Verhältnis 1 erfüllen, und
wobei das warmgewalzte Stahlblech in Fläche 10 bis 30% an Ferrit, 20 bis 40% an Perlit und 35 bis 55 % an Bainit als Mikrostruktur umfasst, $\begin{matrix}0,235 \left[C\right] + 0,0158 \left[Mn\right] + 0,0625 \left[Si\right] + 0,0423 \left[Mo\right] + 0,317 \left[Ti\right] + 1,36 \left[Nb\right] \\ \leq 0,075 ,\end{matrix}$
wobei [C], [Mn], [Si], [Mo], [Ti] und [Nb] den Gehalt der entsprechenden Elemente darstellen, die jeweils in Gew.-% im Stahlblech enthalten sind.

2. Beschichtetes Stahlblech nach Anspruch 1, wobei eine Summe der Fraktionen an Ferrit, Perlit und Bainit 90 Flächen-% oder mehr beträgt.

3. Beschichtetes Stahlblech nach Anspruch 1, wobei eine durchschnittliche Korngröße des Ferrits 20 µm oder weniger beträgt, 0 µm ausgenommen.

4. Beschichtetes Stahlblech nach Anspruch 1, wobei eine durchschnittliche Koloniegröße des Perlits 30 µm beträgt, 0 µm ausgenommen.

5. Beschichtetes Stahlblech nach Anspruch 1, wobei die Plattierungsschicht in Gewicht 10 % oder weniger an Mg, 5 % oder weniger an AI, einen Rest an Zn und unvermeidbare Verunreinigungen umfasst.

6. Beschichtetes Stahlblech nach Anspruch 1, wobei das beschichtete Stahlblech eine Streckgrenze von 450 bis 600 MPa hat.

7. Beschichtetes Stahlblech nach Anspruch 1, wobei das Produkt einer Streckgrenze und einer Dehnung des beschichteten Stahlblechs 8,500 MPa·% oder mehr beträgt.

8. Beschichtetes Stahlblech nach Anspruch 1, wobei das warmgewalzte Stahlblech ein dünnes Material von weniger als 2,0 mm Schichtdicke ist.

9. Verfahren zum Herstellen eines beschichteten Stahlblechs, umfassend:
Wiedererwärmen einer Bramme, die in Gewicht 0,15 bis 0,25% an C, 0,5% oder weniger an Si, 0,5 bis 2,0 % an Mn, 0,03% oder weniger an P, 0,015% oder weniger an S, 0,05% oder weniger an AI, 0,01% oder weniger an N, 0,01 bis 0,05% an Ti, 0,0005 bis 0,01% an B, einen Rest an Eisen und unvermeidbare Verunreinigungen umfasst, auf 1100 bis 1300°C, wobei die Elemente die folgende Gleichung 1 erfüllen;
Fertigwalzen der wiedererwärmten Bramme auf eine Temperatur von Ar3°C oder höher, um ein warmgewalztes Stahlblech zu erhalten;
Abkühlen des warmgewalzten Stahlblechs mit einer Rate von Vc bis (Vc + 30) °C/s, die durch die folgende Gleichung 1 definiert ist, und Aufwickeln des gekühlten, warmgewalzten Stahlblechs; und
Heißtauchbeschichten, indem das aufgewickelte, warmgewalzte Stahlblech in eine Heißtauchbad eingetaucht wird,
wobei das Fertigwalzen in einem Bereich von (FDT - 20) °C bis (FDT + 20) °C ausgeführt wird, der durch die folgende Gleichung 2 definiert ist, und
wobei das Aufwickeln in einem Bereich von (CT - 20) °C bis (CT + 20) °C ausgeführt wird, der durch die folgenden Gleichung 3 definiert ist, $\begin{matrix}0,235 \left[C\right] + 0,0158 \left[Mn\right] + 0,0625 \left[Si\right] + 0,0423 \left[Mo\right] + 0,317 \left[Ti\right] + 1,36 \left[Nb\right] \\ \leq 0,075 ,\end{matrix}$
wobei [C], [Mn], [Si], [Mo], [Ti] und [Nb] den Gehalt der entsprechenden Elemente darstellen, die jeweils in Gew.-% im Stahlblech enthalten sind, $\begin{matrix}Vc = 158,0 - 156,6 \left[C\right] + 246,6 \left[Si\right] - 40,32 \left[Mn\right] - 25,74 \left[Cr\right] - 73,26 \left[Ni\right] - \\ 8820 \left[B\right] - 1483,2 \left[Ti\right] + 1108,8 \left[Nb\right] - 291,6 \left[Mo\right] - 1092,6 \left[V\right] ,\end{matrix}$
wobei [C], [Si], [Mn], [Cr], [Ni], [B], [Ti] [Nb], [Mo] und [V] den Gehalt der entsprechenden Elemente darstellen, die jeweils in Gew.-% im Stahlblech enthalten sind, $\begin{matrix}FDT \left(°C\right) = 1002,1 - 353 \left[C\right] + 43,9 \left[Si\right] - 74,1 \left[Mn\right] - 20,4 \left[Cu\right] - 19,9 \left[Cr\right] - \\ 45,6 \left[Ni\right] - 80 \left[Mo\right] ,\end{matrix}$
wobei [C], [Si], [Mn], [Cu], [Cr], [Ni], und [Mo] den Gehalt der entsprechenden Elemente darstellen, die jeweils in Gew.-% im Stahlblech enthalten sind, $CT = 751,7 - 357,3 \left[C\right] - 85,3 \left[Mn\right] - 35 \left[Si\right] - 73 \left[Cr\right] - 36 \left[Ni\right] - 8,4 \left[Mo\right] ,$
wobei [C], [Mn], [Si], [Cr] [Ni] und [Mo] den Gehalt der entsprechenden Elemente darstellen, die jeweils in Gew.-% im Stahlblech enthalten sind.

10. Verfahren nach Anspruch 9, wobei das Heißtauchbad in Gewicht 10 % oder weniger an Mg, 5 % oder weniger an AI, einen Rest an Zn und unvermeidbare Verunreinigungen umfasst.

## Revendications

1. Tôle d'acier plaquée présentant un film de placage sur une surface d'une tôle d'acier laminée à chaud, sachant que la tôle d'acier laminée à chaud comprend, en poids, 0,15 à 0,25 % de C, 0,5 % ou moins de Si, 0,5 à 2,0 % de Mn, 0,03 % ou moins de P, 0,015 % ou moins de S, 0,05 % ou moins d'Al, 0,01 % ou moins de N, 0,01 à 0,05 % de Ti, 0,0005 à 0,01 % de B, un solde de Fe, et des impuretés inévitables,
sachant que les éléments satisfont à la relation 1 ci-après, et
sachant que la tôle d'acier laminée à chaud comprend, en aire, 10 à 30 % de ferrite, 20 à 40 % de perlite, et 35 à 55 % de bainite, comme microstructure, $\begin{matrix}0,235 \left[C\right] + 0,0158 \left[Mn\right] + 0,0625 \left[Si\right] + , 0423 \left[Mo\right] + 0,317 \left[Ti\right] + 1,36 \left[Nb\right] \leq \\ 0,075 ,\end{matrix}$
sachant que [C], [Mn], [Si], [Mo], [Ti], et [Nb] représentent la teneur des éléments correspondants contenus dans la tôle d'acier en % de poids, respectivement.

2. La tôle d'acier plaquée selon la revendication 1, sachant qu'une somme des fractions de la ferrite, de la perlite, et de la bainite est de 90 % en aire ou plus.

3. La tôle d'acier plaquée selon la revendication 1, sachant qu'une taille de grain moyenne de la ferrite est de 20 µm ou moins à l'exclusion de 0 µm.

4. La tôle d'acier plaquée selon la revendication 1, sachant qu'une taille de colonie moyenne de la perlite est de 30 µm ou moins à l'exclusion de 0 µm.

5. La tôle d'acier plaquée selon la revendication 1, sachant que le film de placage comprend, en poids, 10 % ou moins de Mg, 5 % ou moins d'AI, un solde de Zn, et des impuretés inévitables.

6. La tôle d'acier plaquée selon la revendication 1, sachant que la tôle d'acier plaquée présente une limite d'élasticité de 450 à 600 MPa.

7. La tôle d'acier plaquée selon la revendication 1, sachant qu'un produit d'une limite d'élasticité et d'un allongement de la tôle d'acier plaquée est de 8 500 MPa·% ou plus.

8. La tôle d'acier plaquée selon la revendication 1, sachant que la tôle d'acier laminée à chaud est un matériau mince de moins de 2,0 mm d'épaisseur de tôle.

9. Procédé de fabrication d'une tôle d'acier plaquée, comprenant :
le réchauffage d'une brame comprenant, en poids, 0,15 à 0,25 % de C, 0,5 % ou moins de Si, 0,5 à 2,0 % de Mn, 0,03 % ou moins de P, 0,015 % ou moins de S, 0,05 % ou moins d'Al, 0,01 % ou moins de N, 0,01 à 0,05 % de Ti, 0,0005 à 0,01 % de B, un solde de Fe, et des impuretés inévitables, à 1100 à 1300 °C,
sachant que les éléments satisfont à la relation 1 ci-après ;
le laminage de finition de la brame réchauffée à une température d'Ar3 °C ou supérieure pour obtenir une tôle d'acier laminée à chaud ;
le refroidissement de la tôle d'acier laminée à chaud à un taux de Vc à (Vc + 30) °C/s défini par l'équation 1 ci-après, et le bobinage de la tôle d'acier laminée à chaud refroidie ; et
le placage par immersion à chaud en immergeant la tôle d'acier enroulée et laminée à chaud refroidie dans un bain d'immersion à chaud,
sachant que le laminage de finition est effectué dans une plage de (FDT - 20) °C à (FDT + 20) °C définie par l'équation 2 ci-après, et
sachant que le bobinage est effectué dans une plage de (CT - 20) °C à (CT + 20) °C définie par l'équation 3 ci-après, $\begin{matrix}0,235 \left[C\right] + 0,0158 \left[Mn\right] + 0,0625 \left[Si\right] + 0,0423 \left[Mo\right] + 0,317 \left[Ti\right] + 1,36 \left[Nb\right] \leq \\ 0,075 ,\end{matrix}$
sachant que [C], [Mn], [Si], [Mo], [Ti], et [Nb] représentent la teneur des éléments correspondants contenus dans la tôle d'acier en % de poids, respectivement, $\begin{matrix}Vc = 158,0 - 156,6 \left[C\right] + 246,6 \left[Si\right] - 40,32 \left[Mn\right] - 25,74 \left[Cr\right] - 73,26 \left[Ni\right] - \\ 8820 \left[B\right] - 1483,2 \left[Ti\right] + 1108,8 \left[Nb\right] - 291,6 \left[Mo\right] - 1092,6 \left[V\right] ,\end{matrix}$
sachant que [C], [Si], [Mn], [Cr], [Ni], [B], [Ti], [Nb], [Mo], et [V] représentent la teneur des éléments correspondants contenus dans la tôle d'acier en % de poids, respectivement, $\begin{matrix}FDT \left(°C\right) = 1002,1 - 353 \left[C\right] + 43,9 \left[Si\right] - 74,1 \left[Mn\right] - 20,4 \left[Cu\right] - 19,9 \left[Cr\right] - \\ 45,6 \left[Ni\right] - 80 \left[Mo\right] ,\end{matrix}$
sachant que [C], [Si], [Mn], [Cu], [Cr], [Ni], et [Mo] représentent la teneur des éléments correspondants contenus dans la tôle d'acier en % de poids, respectivement, $CT = 751,7 - 357,3 \left[C\right] - 85,3 \left[Mn\right] - 35 \left[Si\right] - 73 \left[Cr\right] - 36 \left[Ni\right] - 8,4 \left[Mo\right] ,$
sachant que [C], [Mn], [Si], [Cr], [Ni], et [Mo] représentent la teneur des éléments correspondants contenus dans la tôle d'acier en % de poids, respectivement.

10. Le procédé selon la revendication 9, sachant que le bain d'immersion à chaud comprend, en poids, 10 % ou moins de Mg, 5 % ou moins d'AI, un solde de Zn, et des impuretés inévitables.
